

1

2,734,029

## CORROSION PREVENTION METHOD

Richard S. Treseder, Oakland, and Philip J. Raifsnider, Richmond, Calif., assignors to Shell Development Company, Emeryville, Calif., a corporation of Delaware

No Drawing. Application February 2, 1953,  
Serial No. 334,726

9 Claims. (Cl. 252—8.55)

This invention relates to a method of corrosion-inhibition of a ferruginous material, e. g., steel, while in contact with an agitated fluid system of liquid or liquefied phases and an atmosphere of aqueous carbonic acid and/or carbon dioxide. More particularly, the invention applies to corrosion-prevention of metal equipment normally used in operating gas-condensate light gasoline wells, whereby such corrosion-prevention is effected during the conventional operation of these wells.

In recent years, the problem of preventing corrosion of ferruginous materials in the systems indicated above has become very serious. No entirely satisfactory method is known for preventing corrosion of tubing in operating wells under the corrosive conditions indicated above.

It is an object of the present invention to provide an inexpensive and industrially feasible method of corrosion-inhibition of ferruginous metals in a system in which an agitated flowing mixture of non-oxidizing gases, a liquefied hydrocarbon phase and an aqueous carbonic acid phase come in contact with such ferruginous metal. It is another object to overcome the disadvantages of prior art practices peculiar to corrosion-inhibition applied in operation of gas-condensate wells. A further object is to provide an inexpensive and industrially feasible corrosion-inhibition treatment of iron-containing metals contacting the above-specified system as it occurs in the base of an operating gas-condensate well.

Now in accordance with the present invention, it has been found that corrosion which is caused by contact of ferruginous metal with a system of non-oxidizing gases, with an agitated flowing mixture of a liquefied hydrocarbon phase, and with an aqueous carbonic acid phase, can be inhibited by introducing thereto (continuously or intermittently), a minor but corrosion-inhibiting amount of a mixture of "sticking residue" sulphates (apparently alkyl ammonium sulphates) originally existing in the acid sludge which results from the treatment or alkylation of petroleum fractions (especially, petroleum distillates) with concentrated sulfuric acid as more particularly described hereinafter. Further, in accordance with the present invention, it has been noted that such sulphates in their form as extracted from acid sludge are stored or transported in ferruginous containers, such as drums or the like, while in a relatively concentrated state, corrosion may occur prior to the time at which the sulphates are mixed with the rising condensate stream in the oil well. In correcting this shortcoming, it has been found that the addition of a metallic nitrite to the concentrated sulphate mixture followed by heating thereof within a stated temperature range results in a concentrated reaction mixture which exhibits no adverse corrosive effect toward ferruginous containers and which, moreover, exhibits highly satisfactory protective effects when utilized in the proper concentration in gas-condensate wells.

The liquefied hydrocarbon phase in gas-condensate wells normally comprises mixtures of liquid methane, ethane, propane, butane and heavier hydrocarbon condensates up to and including light gasolines having up to

2

about eight carbon atoms. Normally gaseous hydrocarbons are partly liquefied in the well because of the pressures ordinarily existing therein. A typical gas-condensate well produces between five and thirty barrels of a liquefied hydrocarbon phase per million cubic feet of gas (MMCF), at a typical well-head temperature and pressure. The temperatures at the bottom of the well usually range from about 85° C. to about 125° C., average temperatures at the well-head being usually in the range 10 from about 45° C. to about 80° C. Pressures in a condensate well usually range from about 1,000 to about 7,000 pounds per square inch absolute. A typical well may have a bottom-hole pressure of about 2,700 p. s. i. a. and a flowing tubing pressure of about 2,000 p. s. i. a. 15 The pressure increases the ratio of gaseous carbon dioxide (present in condensate wells) which will dissolve in the aqueous phase also present therein. At well-head conditions there is usually a range from about seven to about twenty gallons or higher of liquid water per MMCF of gas produced. This liquid water phase dissolves carbon dioxide thus providing the aqueous carbonic acid phase. The latter usually has a pH value ranging from about 3.3 to about a pH of 5.5. This aqueous phase also may contain sodium chloride and other electrolytes, the usual amounts of which are well known to the art. Aqueous carbonic acid phase mixed with agitated liquefied hydrocarbon phase and gases is usually distributed throughout the flowing system of the well.

20 The inhibitor is indeterminate in character with respect to the isolation of identifiable members. This is, of course, due to the highly complex nature of the components found in the sludge resulting from acid treatment or alkylation petroleum products.

25 A typical process for recovery of the desired amine sulphates comprises the following steps: Acid sludge, such as that derived by treatment of gas oil with concentrated sulfuric acid, is contacted with ammonia in the presence of water to form an aqueous ammonium sulfate solution; treating at least a portion of (i. e. 10-100%) said solution with petroleum nitrogen bases (3-10% by volume) 30 whereby complexes are formed between said bases and the desired organic sulphates; displacement of the bases from the complex by treatment with ammonia, thus obtaining the organic ammonium sulphates.

35 It will be understood that the precise source of the acid sludge and the particular process for the isolation of the subject inhibitors therefrom do not constitute a part of the present invention. One process for such isolation is described in U. S. Patent 2,331,235 to J. D. Ruys wherein the desired inhibitors are referred to as "sticky residue."

40 The described process is especially suitable for extraction of alkylation acid sludges, but may also use petroleum product treating acid sludges as well, wherein the treatment has been either sulfonation or removal of unsaturates, such as the acid treatment of pressure distillates and the like. Other bases instead of ammonia may be employed, such as sodium, potassium or calcium hydroxides. The nitrogen bases capable of forming complexes with the inhibitor may be those isolated from the sludge, such as taught by the Ruys patent. Alternatively, 45 bases such as the picolines or quinolines may be used.

50 Acid sludges contain a complex mixture of sulfuric acid, water, sulfur dioxide, sulfonic acids, nitrogen bases, hydrocarbon materials, alcohols, esters, hydrogen sulfide and ammonium salts of organic sulfuric acids. These are 55 believed to comprise predominantly ammonium salts of alkyl sulfuric acids having the general formula



60 wherein R is an alkyl radical having from about 3 to 70 about 12 carbon atoms, and usually from about 4 to about 8 carbon atoms. The subject sulphates are substan-

tially water dispersable, or soluble in aqueous ammonium sulfate solutions.

Particularly significant corrosion-prevention in the practice of the invention has been obtained with the water-dispersible sulfates obtained from the above-described sources at concentrations below about 1% by weight of the aqueous phase in the gas-condensate well but preferably above about 0.01% by weight thereof.

It is not known just how the present class of inhibitors act to prevent corrosion of steel under the conditions employed in the present invention. Suffice it to say that they have been found to act effectively. This is surprising in view of the turbulence of flow in the system and the low concentrations of inhibitor (less than about 1 wt. per cent, based on the liquefied hydrocarbon phase) which are effective relative to the much higher concentrations of carbonic acid and other dispersing components in the system. Also, these inhibitors are sensitive to the liquefied hydrocarbon phase; so it would seem that they would be swept away by the turbulence flow of this phase, leaving the surface of the metal open to attack by the swiftly churning aqueous carbonic acid present.

The present agents may be introduced into gas-condensate wells in various ways. For example, tubing of relatively small diameter may be run down through the production tube of such a well to approximately the bottom end thereof, and a solution of the present agents may be pumped through the small diameter tubing so as to enter the well stream near the bottom of the well tube; the rising turbulent flow will then carry the injected agent up through the tube. Obviously, the corrosion inhibitors may be added to or introduced into the wells by other means or methods depending, in part, on whether the wells are operated through the casings or through tubing disposed in such casings. Also, it is clear that the inhibitors may be introduced into the top of the well and allowed to flow down, or may be forced to any given point or points in the well, at which the inhibitor then can come in contact with the turbulent up-flowing fluid mixture which, as stated, would cause metal corrosion but for the presence of the corrosion inhibitors of this invention. The inhibitor may be mixed with 10-100% of petroleum waxes to form a solid composition which may be dropped in the well in the form of granules, cubes or sticks.

The employment of the present agents is best effected by having them in solution in an aqueous medium readily miscible with the aqueous phase of the well system, and then introducing the solution of the agent or agents to a condensate well as above-described. Any solvent which is substantially non-reactive with the agents under the conditions employed (e. g., such solvents as esters, alcohols, ketones, etc.) may be used for preparing an inhibitor solution, although it is preferable to employ water. In some cases it is advantageous to use a more or less concentrated solution or dispersion (as up to about 50 wt. per cent of the agent(s)) in a suitable fluid medium. The amount of solvent in the inhibitor solution is so small, relative to the volume of liquid in the system treated therewith, that it does not materially affect the normal operation of the well.

For purposes of further illustration, reference will now be made to the following examples, it being understood that there is no intention of being limited necessarily to the specific conditions disclosed therein. In these examples steel plates (3/8 inch width, 5 1/2 inch length, sand-blasted coldrolled steel strips) were placed in glass oil-sample bottles containing 10 g. of a water solution having 3% wt. per cent of sodium chloride, 0.1% wt. CaCl<sub>2</sub>, 0.03% MgCl<sub>2</sub>, 0.1% acetic acid and 50 ml. of kerosene containing in some cases the additive of the present invention, obtained from alkylation acid sludge. The concentration of the additive was based upon the water content. The contents of each bottle were then saturated with carbon dioxide gas as follows: Air was displaced by passing carbon dioxide to the bottom of each bottle

for approximately 10 minutes. The prepared bottles were then tightly closed and the stoppers wired on to withstand the pressure developed at elevated temperatures. The bottles were then rotated end-over-end at 60 R. P. M. at a temperature of approximately 80° C. for a period ranging from 18 to 24 hours. At the end of this time the corrosion rates were measured for each steel plate. The results obtained by following the above-described technique are given below:

#### Example I

A series of steel plates were subjected to the above treatment in a container having 50 ml. of kerosene and 10 ml. of water, the latter containing 3% by weight of sodium chloride, 0.1 CaCl<sub>2</sub>, 0.1% w. acetic acid and 0.03% w. MgCl<sub>2</sub>. No corrosion inhibitor was present. An analysis of the thus treated plates showed that the average corrosion rate was about .50 mils per year.

#### Example II

Steel plates of the above type were treated in the same manner in the presence of sulfates isolated from acid sludge resulting from the treatment of west coast petroleum distillates. The inhibitor was utilized in amounts of 0.05%, 0.1% and 0.2% by weight of the water phase. After treatment the plates showed that the corrosion resulting from the use of such inhibited combinations was in the order of 10, 8 and 7 mils per year, respectively. Consequently, it will be seen that the rate of corrosion was reduced sharply when the complex mixture of amine sulfates was utilized.

#### Example III

Utilizing the information gained in the above-described laboratory experiments, field trials were instituted in which the complex inhibitor was introduced periodically into the annulus between the well casing and the well tubing. The well being treated was one producing approximately 4.6 million cubic feet gas and condensate per day. The well was yielding approximately 10 barrels of salt water at the same time. The corrosion rate of the test panels exposed in the floor line of the well dropped from 110 mils per year when the well was uninhibited to about 10 mils per year at the end of a six-weeks' period, the injection rate being about 0.4 quart of inhibitor per million cubic feet of gas condensate, or about 0.12% based on the water phase.

#### Example IV

Due to the occurrence of a certain amount of corrosion in iron drums in which the concentrated inhibitor was stored and transported, the amine sulfate mixture was modified by the following process:

3215 lbs. of "sticky residue" organic ammonium sulfates from refinery acid sludge, having a pH of 2.0, was neutralized to pH of 6.8 by the addition of 89 lbs. of anhydrous ammonia. Sodium nitrite amounting to 195 lbs., or 6% by weight of the charge, was then added and the mixture stirred at 55-60° C. for 17 hours. Following this reaction period (during which a portion of the sodium nitrite was converted to nitrous acid) the charge was cooled without stirring and settled for four days. A lower phase consisting mainly of ammonium sulfate was run off to waste while the upper oily phase, weighing 2615 lbs., was transferred to drums. The resulting concentrated and inhibited mixture of amine sulfates exhibited no corrosion of the iron drums during an extended storage and shipping period.

The treatment of the sludge sulfates derived from petroleum refinery acid sludges preferably comprises the addition of between about 0.1 and about 50% of a metallic nitrite based on the weight of concentrated amines, said concentrated amines constituting approximately between about 10% and about 80% of sludge sulfates. In order to produce the desired reaction between the nitrite and the crude sulfate mixture heating is preferably conducted

at temperatures between about 40° C. and 80° C. for periods of between about one-half hour and 72 hours. The resulting mixture preferably contains a residual amount of sodium nitrite in the order of about .01-2.0% based on the concentrated amine sulfates, the remainder having been converted to nitrous acid which eventually is dispersed from the system in the form of nitrogen oxides and water. This inhibited concentrate was then employed in a well injection as described in the previous example to obtain a substantial reduction in corrosion.

We claim as our invention:

1. The method of treating a hydrocarbon-containing system in its natural state in a well for the purpose of inhibiting corrosion by aqueous carbonic acid of well metal parts, said system comprising a non-oxidizing gas phase, a liquefied normally gaseous hydrocarbon phase and a minor amount of aqueous carbonic acid, which system in a state of agitated flow at a temperature of between about 45° C. and about 125° C. and under a pressure of between about fifteen and seven thousand pounds per square inch absolute, comes in contact with corrodible well parts, which method includes the step of mixing with said system an amount of below approximately one weight per cent and above approximately 0.0001 weight per cent of the liquid hydrocarbon phase contacted, of water soluble ammonium salts of organic sulfuric acids isolated from petroleum refinery acid sludge.

2. The method of treating a hydrocarbon-containing system in its natural state in a well for the purpose of inhibiting corrosion by aqueous carbonic acid of well metal parts, said system comprising a non-oxidizing gas phase, a liquefied normally gaseous hydrocarbon phase and a minor amount of aqueous carbonic acid, which system in a state of agitated flow at a temperature of between about 45° C. and about 125° C. and under a pressure of between about fifteen and seven thousand pounds per square inch absolute, comes in contact with corrodible well parts, which method includes the step of mixing with said system an amount of below about 1% by weight and above about 0.0001% by weight of the aqueous phase contacted of water-dispersible ammonium salts of organic sulfuric acids, said sulfates being those recovered from the acid sludge resulting from the sulfuric treatment of petroleum distillates, said sulfates also containing between about 0.01% and about 2.0% by weight thereof of a metallic nitrite.

3. A process according to claim 2 wherein the nitrite is an alkali metal nitrite.

4. A process according to claim 2 wherein the nitrite is sodium nitrite.

5. A process according to claim 1 wherein the acid sludge is that resulting from the alkylation of petroleum distillates with sulfuric acid.

6. A process according to claim 1 wherein the ammonium salts are those obtained by the treatment of petroleum distillates in the kerosene and gas oil ranges with sulfuric acid for the removal of unsaturated hydrocarbons.

7. The method of treating a hydrocarbon-containing system in its natural state in a well for the purpose of inhibiting corrosion by aqueous carbonic acid of well metal parts, said system comprising a non-oxidizing gas

10 phase, a liquefied normally gaseous hydrocarbon phase and a minor amount of aqueous carbonic acid, which system in a state of agitated flow at a temperature of between about 45° C. and about 125° C. and under a pressure of between about fifteen and seven thousand pounds per square inch absolute, comes in contact with corrodible well parts, which method includes the step of mixing with said system an amount of below about 1% by weight and above about 0.0001% by weight of the aqueous phase contacted of water-dispersible ammonium salts of alkyl sulfuric acids, said sulfates being those recovered from the acid sludge resulting from the sulfuric treatment of petroleum distillates, said sulfates also containing between about 0.1% and about 2.0% by weight thereof of a metallic nitrite.

15 20 25 8. A process according to claim 7 in which the alkyl radicals of the ammonium salts of alkyl sulfuric acids predominates in radicals having from 3 to 12 carbon atoms each.

20 25 30 35 40 45 9. In the method of improving the corrosion properties of water-dispersible ammonium salts of alkyl sulfuric acids, said salts being recovered from the acid sludge resulting from the sulfuric acid treatment of petroleum distillates, and said sulfates being corrosive in concentrated solution toward ferruginous metals, the steps comprising adding to said ammonium salts an amount between about 0.1 and about 50% by weight of a metallic nitrite based on the crude salt mixture, said mixture comprising between about 10% and about 80% by weight of ammonium salts, and heating the mixture of ammonium salts and nitrite at a temperature between about 40° C. and 80° C. for a period between about one-half and about 72 hours, the resulting mixture containing between about 0.01 and 2.0% by weight of metallic nitrite subsequent to said heating period.

References Cited in the file of this patent

UNITED STATES PATENTS

|           |                      |               |
|-----------|----------------------|---------------|
| 2,331,235 | Ruys et al. -----    | Oct. 5, 1943  |
| 2,402,793 | White et al. -----   | June 25, 1946 |
| 2,582,733 | Zimmer et al. -----  | Jan. 15, 1952 |
| 2,583,399 | Wachter et al. ----- | Jan. 22, 1952 |